

# United States Patent Office

2,851,420

Patented Sept. 9, 1958

1

2,851,420

## SALT BATHS, METHOD OF MAINTAINING SALT BATHS NEUTRAL, AND ADDITIVE THEREFOR

Artemas F. Holden, Milford, Mich.

No Drawing. Application July 14, 1955  
Serial No. 522,176

9 Claims. (Cl. 252—71)

This invention relates to a molten salt bath containing a novel combination of ingredients whereby the efficiency of the bath is maintained over long periods of use. The invention further relates to a method of reconstituting neutral salt baths and to a novel additive for such purpose. This application is a continuation-in-part of my patent application S. N. 317,365, filed October 28, 1952, now abandoned.

Neutral salt baths, which often comprise chlorides of the alkali metals and alkaline earth metals with or without fluorides of these metals, are commonly used in industry for the heating of metals, as for instance during their heat treatment. It is well known that, after a period of use, initially neutral baths become alkaline and thus decarburizing to steel due to breakdown of the salts at elevated temperature.

It has been common in the industry to rectify neutral salt baths by adding thereto rectifiers containing either silica, titanium dioxide, silicon carbide, borax, or boric acid. These rectifiers react with the salts to form residual sludges which are basically ceramic in nature. The metal oxides react with these ceramic materials and are separated from the salt bath and enter into a water-insoluble sludge.

Where borax or boric acid is used as a rectifier, either singly or in combination, these components combine with the alkali and metal oxides to form sludges of a more or less glassy type. The action of any of the previously mentioned rectifiers is not sustained but very temporary in character; and, in addition, when rectifiers containing boric acid are added to a molten salt bath, a viscous liquid is formed on the top surface of the bath which persists for a period of from 5 to 20 minutes after addition of the rectifier. The salt bath cannot then be used until total destruction of the boric acid and assimilation of the viscous liquid. Moreover, it is necessary from time to time to remove the residual sludges which, if permitted to remain in the bath, tend to increase viscosity of the bath and are water-insoluble so as to be difficult to wash from the heat treated parts.

I have found that when a composition termed "magnesium boron fluoride" and consisting essentially of a complex salt of magnesium fluoride, boric oxide, and water and having the approximate formula



is added to neutral salt baths composed of salts of the alkali metals and alkaline earth metals, with or without smaller amounts of fluorides of these metals, in amounts between 0.25% and 4% by weight of the total bath, this material is readily assimilated into the bath at a range of temperatures between 840° F. and 2400° F. Magnesium boron fluoride may be added to the bath either initially or after the bath has become contaminated by normal breakdown of the salts from use and will reduce and hold the water insolubles, acid insolu-

2

bles, and metal oxides to a minimum and maintain the bath in neutral condition.

It is believed that this composition operates through its slow reaction under the effect of elevated temperatures, such as those employed in the above-mentioned baths. The reaction appears to have the effect of releasing compounds within the bath which react with the metal oxides and with breakdown products of the salts and prevent attack on or decarburization of metals in the bath. Another reaction is believed to take place between the metal oxides and boric anhydride, released by the composition, resulting in insoluble metal pyroborates.

In a bath of the type above described containing the additive of the present invention, the electrodes of the direct-resistance type of salt bath furnace employing immersed electrodes have a much longer life and the life of the pot of a ceramic pot electrode furnace is increased substantially.

Magnesium boron fluoride, which is currently manufactured by the American Agricultural Chemical Company, may be made by mixing magnesium fluoride and orthoboric acid in the solid state in the ratio of four moles of magnesium fluoride to one mole of orthoboric acid and heating the mixture at atmospheric pressure to about 190° C. The reaction produces a complex salt having the approximate formula



The amount of water left in the magnesium boron fluoride may be expected to vary with the duration of the molten condition of the orthoboric acid. The actual component may be from 1½ to 2½ moles of water of water of hydration. Magnesium boron fluoride, as manufactured by American Agricultural Chemical Company, falls within the following partial analysis:

|                  | Percent by weight |
|------------------|-------------------|
| Magnesium        | 25½-27            |
| Boron            | 5.7-5.9           |
| Fluorine         | 33-36             |
| Loss on ignition | 8½-12             |

This calculates to:

|                                                               | Percent by weight |
|---------------------------------------------------------------|-------------------|
| MgF <sub>2</sub>                                              | 67-70             |
| B <sub>2</sub> O <sub>3</sub>                                 | 18-19             |
| Water (preferably)                                            | 9-12              |
| Other (lime, silica, sulfate, fluoride, iron, oxide, alumina) | Trace to about 2  |

A presently used composition of the material is approximately as follows:

|                                                               | Percent by weight |
|---------------------------------------------------------------|-------------------|
| Magnesium fluoride                                            | 69.5              |
| Boric oxide                                                   | 18.5              |
| Water (combined and free)                                     | 10.0              |
| Other (lime, silica, sulfate, fluoride, iron, oxide, alumina) | 2                 |

The two percent of miscellaneous impurities present in the ore (such as sellaite) do not appear to have any effect, beneficial or otherwise, either in the manufacture of magnesium boron fluoride or its use as an additive for salt baths.

The following examples of molten salt baths within the scope of the invention are given by way of illustration. It is to be understood that the invention is not to be limited to these specific examples, either as it relates to the relative amount of the ingredients in the bath or to the basic composition of the bath to which the magnesium boron fluoride is added, the scope of the invention being defined by the claims appended hereto.

## EXAMPLE NO. 1.—NEUTRAL PREHEATING BATH

This bath had the following initial composition:

|                          | Percent by weight |
|--------------------------|-------------------|
| Barium chloride          | 49                |
| Potassium chloride       | 25                |
| Sodium chloride          | 25                |
| Magnesium boron fluoride | 1                 |

This bath is suitable for use at an operating range of 1200° F. to 1700° F. When used at slightly above its melting point, 1/4 percent of magnesium boron fluoride is all that is required due to slow breakdown of the salts by contact with the atmosphere. The bath is also operable at higher temperatures and may be used at operating temperatures up to 1700° F. This bath was employed (1) as a first preheat bath for high-speed steels operating at about 1400° F. and (2) a second preheat bath for high-speed steels operating at about 1550° F. The baths were operated continuously in the usual manner for a

4  
of either of the examples other than addition of bath of the initial composition to make up for losses due to drag-out of the bath on fixtures and parts being treated.

## EXAMPLE NO. 2.—NEUTRAL HIGH HEAT BATH

This bath had the following initial composition:

|                          | Percent by weight |
|--------------------------|-------------------|
| Barium chloride          | 96                |
| Magnesium boron fluoride | 4                 |

10 This salt bath was continuously operated in conjunction with the previously mentioned preheat baths in the heat treatment of high-speed steels, the bath being operated at temperatures of 2200° F. to 2300° F. This bath was tested at intervals similarly to the bath of Example 1. 15 There were no additions to the bath other than salt bath carried over from the preheat baths and addition of bath of the initial composition of Example No. 2 to make up for normal consumption due to drag-out.

The results of the tests of the baths of Examples 1 and 2 are as follows:

| Bath              | Date    | Neutral Test, ml./1 gr. | Water Insol., Percent | Acid Insol., Percent | Metal Oxides, Percent | Other, Percent              |
|-------------------|---------|-------------------------|-----------------------|----------------------|-----------------------|-----------------------------|
| #1PH (Ex. 1)----- | 1-14-AM | 0.4                     | 0.44                  |                      |                       |                             |
|                   | 1-14-PM | 0.5                     | 0.40                  |                      |                       |                             |
|                   | 1-17-AM | 0.3                     | 0.54                  | avg. 0.01            | avg. 0.07             |                             |
|                   | 1-17-PM | 0.4                     | 0.46                  |                      |                       |                             |
|                   | 1-18-AM | 0.4                     | 0.63                  |                      |                       |                             |
|                   | 1-18-PM | 0.5                     | 0.54                  |                      |                       |                             |
|                   | 1-14-AM | 0.2                     | 0.61                  |                      |                       |                             |
|                   | 1-14-PM | 0.3                     | 0.45                  |                      |                       |                             |
|                   | 1-17-AM | 0.3                     | 0.41                  |                      |                       |                             |
|                   | 1-17-PM | 0.4                     | 0.46                  |                      |                       |                             |
| #2PH (Ex. 1)----- | 1-18-AM | 0.3                     | 0.40                  |                      |                       |                             |
|                   | 1-18-PM | 0.3                     | 0.54                  |                      |                       |                             |
|                   | 1-14-AM | 0.7                     | 0.49                  |                      |                       |                             |
|                   | 1-14-PM | 1.0                     | 0.70                  |                      |                       |                             |
|                   | 1-17-AM | 1.5                     | 1.20                  |                      |                       |                             |
|                   | 1-17-PM | 1.8                     | 0.87                  | avg. 0.025           | avg. 0.063            |                             |
|                   | 1-18-AM | 2.0                     | 0.95                  |                      |                       |                             |
|                   | 1-18-PM | 1.7                     | 1.32                  |                      |                       |                             |
|                   | 1-21-AM | 0.4                     | 0.41                  |                      |                       |                             |
|                   | 1-22-PM | 0.4                     | 0.43                  |                      |                       |                             |
| #HH (Ex. 2)-----  | 1-24-AM | 0.5                     | 0.45                  | avg. 0.02            | avg. 0.13             |                             |
|                   | 1-24-PM | 0.5                     | 0.28                  |                      |                       |                             |
|                   | 1-25-AM | 0.3                     | 0.40                  |                      |                       |                             |
|                   | 1-25-PM | 0.4                     | 0.37                  |                      |                       |                             |
|                   | 1-21-AM | 0.4                     | 0.81                  |                      |                       |                             |
|                   | 1-22-PM | 0.4                     | 0.44                  |                      |                       |                             |
|                   | 1-24-AM | 1.9                     | 0.50                  |                      |                       |                             |
|                   | 1-24-PM | 1.9                     | 0.52                  | avg. 0.02            | avg. 0.04             | MoO <sub>3</sub> avg. 0.08  |
|                   | 1-25-AM | 2.2                     | 0.51                  |                      |                       |                             |
|                   | 1-25-PM | 1.9                     | 0.60                  |                      |                       |                             |
| #1PH (Ex. 1)----- | 1-29-AM | 0.3                     | 0.45                  |                      |                       |                             |
|                   | 1-29-PM | 0.4                     | 0.45                  |                      |                       |                             |
|                   | 1-31-AM | 0.4                     | 0.45                  | avg. 0.021           | avg. 0.13             | MoO <sub>3</sub> trace only |
|                   | 1-31-PM | 0.5                     | 0.45                  |                      |                       |                             |
|                   | 2-2-AM  | 0.5                     | 0.45                  |                      |                       |                             |
|                   | 2-2-PM  | 0.5                     | 0.41                  |                      |                       |                             |
|                   | 1-29-AM | 0.4                     | 0.84                  |                      |                       |                             |
|                   | 1-29-PM | 0.45                    | 0.80                  |                      |                       |                             |
|                   | 1-31-AM | 0.4                     | 0.95                  | avg. 0.066           | avg. 0.055            | MoO <sub>3</sub> 0.01       |
|                   | 1-31-PM | 0.4                     | 0.87                  |                      |                       |                             |
| #2PH (Ex. 1)----- | 2-2-AM  | 0.4                     | 0.83                  |                      |                       |                             |
|                   | 2-2-PM  | 0.4                     | 0.78                  |                      |                       |                             |
|                   | 1-29-AM | 1.8                     | 0.44                  |                      |                       |                             |
|                   | 1-29-PM | 1.1                     | 0.62                  |                      |                       |                             |
|                   | 1-31-AM | 1.8                     | 0.42                  | avg. 0.14            | avg. 0.11             | MoO <sub>3</sub> 0.03       |
|                   | 1-31-PM | 1.8                     | 0.70                  |                      |                       |                             |
|                   | 2-2-AM  | 2.1                     | 0.44                  |                      |                       |                             |
|                   | 2-2-PM  | 2.3                     | 0.51                  |                      |                       |                             |
|                   | 1-31-AM | 1.8                     | 0.42                  | avg. 0.066           | avg. 0.14             | avg. nil.                   |
|                   | 1-31-PM | 1.8                     | 0.70                  |                      |                       |                             |
| #HH (Ex. 2)-----  | 2-2-AM  | 2.1                     | 0.44                  |                      |                       |                             |
|                   | 2-2-PM  | 2.3                     | 0.51                  |                      |                       |                             |
|                   | 1-31-AM | 1.8                     | 0.42                  |                      |                       |                             |
|                   | 1-31-PM | 1.8                     | 0.70                  |                      |                       |                             |
|                   | 2-2-AM  | 2.1                     | 0.44                  |                      |                       |                             |
|                   | 2-2-PM  | 2.3                     | 0.51                  |                      |                       |                             |
|                   | 1-31-AM | 1.8                     | 0.42                  |                      |                       |                             |
|                   | 1-31-PM | 1.8                     | 0.70                  |                      |                       |                             |
|                   | 2-2-AM  | 2.1                     | 0.44                  |                      |                       |                             |
|                   | 2-2-PM  | 2.3                     | 0.51                  |                      |                       |                             |

period of twenty days in the preheating of high-speed steel. During this time samples were taken at intervals and one gram of each sample was titrated with 10/N hydrochloric acid with methyl red as an indicator. The following table indicates the time of sampling and the amount of 10/N hydrochloric acid required, thus indicating the degree of alkalinity of the bath. The acid insolubles, water insolubles, and other elements were determined by standard chemical analysis. During the period of these tests, there were no additions to the baths

The following specific examples of salt bath compositions have also been used successfully:

EXAMPLE NO. 3.—HARDENING BATH  
(Operating Range 1000° F. to 1550° F.)

|                          | Percent |
|--------------------------|---------|
| Sodium chloride          | 25      |
| Barium chloride          | 30      |
| Calcium chloride         | 44      |
| Magnesium boron fluoride | 1       |

EXAMPLE NO. 4.—HARDENING BATH  
(Operating Range 1250° F. to 1650° F.)

|                          |    |
|--------------------------|----|
| Potassium chloride       | 44 |
| Sodium chloride          | 45 |
| Sodium fluoride          | 6  |
| Barium chloride          | 5  |
| Magnesium boron fluoride | 1  |

EXAMPLE NO. 5.—HARDENING BATH  
(Operating Range 1450° F. to 2000° F.)

|                          |      |
|--------------------------|------|
| Barium chloride          | 77   |
| Calcium chloride         | 16.5 |
| Sodium fluoride          | 5.5  |
| Magnesium boron fluoride | 1    |

The use of magnesium boron fluoride as above described in high-temperature salt baths heated with immersed electrodes of Inconel and type 446 chrome electrode metal appears to greatly prolong the electrode life. It has been observed that a bath containing magnesium boron fluoride will tend to reduce chrome oxide to metallic chromium on the surface of the electrodes so as to build up an outer layer of high chromium concentration, which in the case of a 2" x 4" chrome electrode bar formed a high chromium layer of  $\frac{1}{8}$ " or more after two months' operation. While Inconel electrodes formerly had a life expectancy of five weeks when used with neutral chloride salt baths at operating temperatures of 2000° F. to 2300° F., in such baths incorporating magnesium boron fluoride a total life of five to seven months of the same electrodes can be expected. It would appear that in each instance the chromium is reduced and forms a high-chrome outer layer so as to protect the nickel or iron content of the metal from attack by the salt bath.

The usual refractory ceramic pots, including those made of mullite and silica-aluminum refractories, are eroded by the baths due largely to abrasion from metal oxides and other inert compounds of rectifiers. Magnesium boron fluoride does not react with the refractory to decrease pot life, but actually enhances life of the refractory due to reduction of oxide content and less sludge.

In accordance with the invention, marked advantages are realized when magnesium boron fluoride is employed in molten baths consisting of chlorides of one or more of the alkali and alkaline earth metals and with other fluorides at temperatures below 2000° F. where scale is present on the parts being processed. It is apparent from tests that other fluorides are helpful, in amounts of 1% to 20%, i. e., sodium, potassium, barium, calcium, or chromium fluoride, depending on temperature and the process for which the ultimate compound is to be used. Magnesium boron fluoride has been found useful with all chloride-fluoride salt baths.

Magnesium boron fluoride also may be added in amounts from  $\frac{1}{4}\%$  to 4% by weight to neutral baths consisting essentially of hydroxides or carbonates of the alkali and alkaline earth metals and to baths consisting essentially of mixtures of such hydroxides, carbonates, and chlorides, or of chlorides and hydroxides, chlorides and carbonates, or hydroxides and carbonates, all of the alkali and alkaline earth metals, with or without fluorides of the alkali and alkaline earth metals present. Magnesium boron fluoride in the percentage range above stated

has been added to the salt bath consisting of an eutectic mixture (about 50%–50%) of potassium hydroxide and sodium hydroxide with beneficial results in the annealing of gold at a temperature of 1000° F. After quenching in water, the gold when subsequently heated to red heat over open flame showed no tarnish, whereas, under such conditions, a definite tarnish was evident when similarly treated in such a bath in which magnesium boron fluoride was not present.

10 I claim:

1. A non-aqueous salt bath composition for the heat treatment of metals at temperatures in excess of 840° F., consisting essentially of a mixture of alkali metal and alkaline earth metal halides which normally break down in use to form metal oxides and hydroxides, and from  $\frac{1}{4}\%$  to 4% by weight of a salt having substantially the formula  $4\text{MgF}_2 \cdot \text{B}_2\text{O}_3 \cdot 2\text{H}_2\text{O}$ .

2. A non-aqueous salt bath composition for the heat treatment of metals at temperatures in excess of 840° F., consisting essentially of a mixture of salts selected from the group consisting of alkali and alkaline earth chlorides, up to 16% by weight of a fluoride selected from the alkali and alkaline earth fluorides, and from  $\frac{1}{4}\%$  to 4% by weight of a salt having the formula



where X can vary from  $1\frac{1}{3}$  to  $2\frac{1}{3}$ .

3. A non-aqueous salt bath composition for the heat treatment of metals at temperatures in excess of 840° F., consisting essentially of at least two salts selected from the alkali and alkaline earth halides, and from  $\frac{1}{4}\%$  to 4% by weight of a salt having the formula



where X can vary from  $1\frac{1}{3}$  to  $2\frac{1}{3}$ .

4. A bath as defined in claim 2, in which at least 80% by weight of the bath is composed of a mixture of at least two chlorides selected from the alkali and alkaline earth chlorides.

5. A bath as defined in claim 3, in which at least two salts are chlorides.

6. A bath as defined in claim 3, in which at least two salts are potassium chloride and sodium chloride.

7. The method of stabilizing a non-aqueous metal heat treating salt bath containing alkali and alkaline earth halides tending to break down in use at temperatures in excess of 840° F. to form the corresponding oxides and hydroxides, comprising adding to the bath a salt having the formula  $4\text{MgF}_2 \cdot \text{B}_2\text{O}_3 \cdot \text{XH}_2\text{O}$ , where X can vary from  $1\frac{1}{3}$  to  $2\frac{1}{3}$ , the addition being in such quantities as to maintain the bath substantially free of the breakdown products.

8. The method of claim 7, in which the salt is added in an amount equivalent to from  $\frac{1}{4}\%$  to 4% of the bath by weight.

9. The method of claim 7, in which the salt bath consists essentially of at least one chloride selected from the group consisting of alkali and alkaline earth chlorides.

60 65 References Cited in the file of this patent

UNITED STATES PATENTS

- 2,510,650 Newell ----- June 6, 1950  
2,620,310 Albrecht ----- Dec. 2, 1952